

# United States Patent Office

2,800,491

1

2,800,491

## **OXIDATION-RESISTANT OLEAGINOUS MATERIALS**

Warren C. Ellis, Jr., Columbus, Ohio, assignor, by mesne assignments, to Stauffer Chemical Company, New York, N. Y., a corporation of Delaware

**No Drawing. Application December 14, 1954,  
Serial No. 475,309**

**18 Claims. (Cl. 260—398.5)**

This invention relates to a method of stabilizing oleaginous materials such as fats, fatty acids and hydrocarbons and to such compounds containing small amounts of stabilizing agents as novel compositions of matter.

As is well-known, oleaginous materials absorb oxygen upon standing for any length of time and become dark and foul smelling. Many attempts have been made in the past to provide antioxidants which will render such materials resistant to oxidation for extended periods of time and at elevated temperatures but ordinarily such agents as have been proposed in the past are not fully effective and must be used in relatively large quantities.

According to the present invention, it has been found that rhodanines, including rhodanine itself and various substituted rhodanines, are very effective as antioxidants for oleaginous materials. At the relatively low concentration of 0.025% by weight, rhodanine renders commercial stearic acid virtually oxidation-proof. Although the substituted rhodanines are not as effective as rhodanine itself, these compounds do possess definite antioxidant properties and in some applications may even be preferred to rhodanine. By using rhodanine as an antioxidant, fatty acids such as commercial stearic acid (a mixture of stearic and palmitic acids) may be kept from developing rancidity and/or peroxides for practically any length of time desired, regardless of whether the fatty acids are maintained in the solid or liquid state, or in the presence or absence of air. Similarly, the rhodanines can be used to stabilize fats, such as lard oil and hydrocarbons such as paraffin wax.

Although rhodanine by itself is very effective, in some situations it has been found that rhodanine may be advantageously combined with other antioxidants to produce even superior results.

2

The rhodanines of the present invention possess the following structural formula:



In the above formula,  $R_1$  and  $R_2$  may be hydrogen atoms, in which case the compound is rhodanine itself, or  $R_1$  and  $R_2$  can be various organic substituents such as 10 alkyl, aryl, alkaryl, aralkyl, or heterocyclic radicals. However, in carrying out the present invention, rhodanine itself is preferred because of its relatively low cost and effectiveness.

In order to test the compounds of the present invention, various fats, fatty acids and paraffin wax were subjected to the Modified Swift Stability Test (active oxygen method). This method is described in Oil and Soap, 22, 101 (1945), and in J. Am. Oil Chem. Soc., 25, 42 (1948). In this test, air is bubbled continuously through a 20 ml. sample which may or may not contain an antioxidant, and maintained at 97.7° C. The air rate is about 130 ml./min. Periodically, small portions of the sample are removed and the peroxide number of the portion determined. The magnitude of the peroxide number is a recognized index of the extent to which undesirable oxidation of the sample has occurred and, therefore, inversely reflects the effectiveness of the antioxidant which may be present in the sample. A peroxide number of about 25 to 35 milliequivalents per kilogram (meq./kg.) is the maximum tolerable for most uses of fatty acids; discoloration and/or rancidity usually become apparent at about this point. Accordingly, it is obvious that different antioxidants may be easily compared on the bases of the induction periods of the samples (or time to first appearance of peroxides), and time for the sample to attain a peroxide number in the range of 25-35 meq./kg. It is also obvious that the longer the induction period and/or the time to maximum tolerable peroxide number, the more effective and valuable the antioxidant. It is obvious that the highest value is attached to an antioxidant which can prevent appearance of any peroxides and rancidity for any desired length of time.

The specific rhodanine-type compounds tested were as follows:

Rhodanine  
3-p-hydroxyphenylrhodanine  
5-methylrhodanine  
3-n-butylrhodanine  
5-furfurylidenerhodanine  
3-methyl-5-ethylrhodanine

The data obtained are as follows:

| Fatty Material                 | Antioxidant                       | Conc., Percent | Induction Period, Hrs. | Time to Reach Peroxide No. of 35 meq./kg., hrs. |
|--------------------------------|-----------------------------------|----------------|------------------------|-------------------------------------------------|
| Stearic Acid <sup>1</sup>      | {None.....                        |                | 0                      | 10                                              |
|                                | Tenox BHA <sup>2</sup> .....      | 0.025          | 16                     | 40                                              |
|                                | 3-p-hydroxy-phenyl rhodanine..... | 0.025          | 0                      | 18                                              |
|                                | 5-methyl-rhodanine.....           | 0.025          | 0                      | 28                                              |
|                                | 3-n-butyl-rhodanine.....          | 0.025          | 0                      | 56                                              |
|                                | 5-furfurylidene-rhodanine.....    | 0.025          | 20                     | 80                                              |
|                                | 3-methyl-5-ethylrhodanine.....    | 0.025          | 42                     | 80                                              |
| Lily Stearic Acid <sup>3</sup> | {Rhodanine.....                   | 0.025          | 336                    |                                                 |
|                                |                                   |                |                        | (25 meq./kg., hrs.)                             |
|                                | {Proprietary.....                 | ?              | 42                     | 90                                              |
|                                | Rhodanine.....                    | 0.005          | 52                     | 180                                             |
|                                | do.....                           | 0.010          | 52                     | 140                                             |
| Oleic Acid                     | do.....                           | 0.025          | 100                    |                                                 |
|                                |                                   |                |                        | (20 meq./kg., min.)                             |
|                                | {None.....                        |                | 0                      | 45                                              |
| Lard Oil                       | Rhodanine.....                    | 0.025          | 0                      | 105                                             |
|                                | {3-n-butyl rhodanine.....         | 0.025          |                        | 8                                               |
|                                | 3-methyl-5-ethylrhodanine.....    | 0.025          |                        | 8                                               |
| Paraffin wax                   | {None.....                        |                |                        | 4½                                              |
|                                | Rhodanine.....                    | 0.1            |                        |                                                 |
|                                | do.....                           | 0.5            |                        |                                                 |

<sup>1</sup> Triple press stearic acid, about 60% stearic and 40% palmitic acids.

<sup>2</sup> Tenox BHA, butylated hydroxyanisole, Tennessee-Eastman Corporation.

<sup>3</sup> Lily stearic acid, Emery Industries, Inc.

The data show that rhodanine is an exceptionally good antioxidant, particularly for saturated fatty acids. No significant amount of peroxides or rancidity could be detected in any of the samples containing 0.025% rhodanine, regardless of the length of time the tests were run. Lower concentrations are somewhat less effective, although still useful, as shown by comparison with the data for Tenox BHA, and for Lily Stearic Acid without additional antioxidant. Rhodanine is less effective at 0.025% as an antioxidant for unsaturated fatty acids (e. g., oleic acid), than for saturated fatty acids.

Fatty acids which can be stabilized in accordance with the present invention include both saturated acids having the formula  $C_nH_{2n+1}COOH$ , and unsaturated fatty acids having the formula  $C_nH_{2n-1}COOH$ , in both cases  $n$  being a number from 6 to 22. Typical fatty acids which may be stabilized include but are not limited to: caprylic, capric, lauric, palmitic, oleic, stearic, capronic, myristic, arachidic, petroselinic, vaccenic, eleostearic, licamic, parinaric, gadoleic, arachiodonic and cetoleic acids.

I claim:

1. The process of stabilizing a member selected from the group consisting of fatty acids, fats, and paraffin wax comprising adding thereto a rhodanine of the formula



wherein  $R_1$  and  $R_2$  are selected from the group consisting of hydrogen atoms, alkyl, aryl, alkaryl, aralkyl and heterocyclic organic radicals.

2. The process of stabilizing a member selected from the group consisting of fatty acids, fats, and paraffin wax comprising adding thereto rhodanine.

3. The process of stabilizing a member selected from the group consisting of fatty acids, fats, and paraffin wax comprising adding thereto 3-o-hydroxyphenyl rhodanine.

4. The process of stabilizing a member selected from the group consisting of fatty acids, fats, and paraffin wax comprising adding thereto 5-methyl rhodanine.

5. The process of stabilizing a member selected from

| Induction Period, Days | After 65 days    |          |
|------------------------|------------------|----------|
|                        | Color            | Acid No. |
| 12                     | Orange.....      | 100.6    |
| 50                     | Pale yellow..... | 38.0     |
| 62                     | White.....       | 2.2      |

35 the group consisting of fatty acids, fats, and paraffin wax comprising adding thereto 3-n-butyl rhodanine.

6. The process of stabilizing a member selected from the group consisting of fatty acids, fats and paraffin wax comprising adding thereto 3-methyl-5-ethyl rhodanine.

40 7. The process of stabilizing commercial stearic acid comprising adding thereto about 0.025% by weight of rhodanine.

8. The process of stabilizing a mixture containing 45 stearic and palmitic acids comprising adding thereto about 0.025% rhodanine.

9. The process of stabilizing paraffin wax comprising adding thereto a small amount of rhodanine.

10. As a new composition of matter, a mixture of 50 a member selected from the group consisting of fatty acids, fats and paraffin wax and a rhodanine of the formula



55 wherein  $R_1$  and  $R_2$  are selected from the group consisting of hydrogen atoms, alkyl, aryl, alkaryl, aralkyl and heterocyclic organic radicals.

11. As a new composition of matter, a member selected from the group consisting of fatty acids, fats, and paraffin wax and rhodanine.

60 12. As a new composition of matter, a mixture of a member selected from the group consisting of fatty acids, fats, and paraffin wax and 3-o-hydroxyphenyl rhodanine.

13. As a new composition of matter, a mixture of 65 a member selected from the group consisting of fatty acids, fats, and paraffin wax and 5-methyl rhodanine.

14. As a new composition of matter, a mixture of a member selected from the group consisting of fatty acids, fats, and paraffin wax and 3-n-butylrhodanine.

70 15. As a new composition of matter, a mixture of a member selected from the group consisting of fatty

acids, fats, and paraffin wax and 3-methyl-5-ethyl rhodanine.

16. As a new composition of matter, commercial stearic acid containing about 0.025% by weight rhodanine.

17. As a new composition of matter, a mixture of stearic and palmitic acids containing about 0.025% rhodanine.

18. As a new composition of matter, paraffin wax containing a small amount of rhodanine.

References Cited in the file of this patent

5 UNITED STATES PATENTS

2,469,378 Flett ----- May 10, 1949

UNITED STATES PATENT OFFICE  
CERTIFICATE OF CORRECTION

Patent No. 2,800,491

July 23, 1957

Warren C. Ellis, Jr.

It is hereby certified that error appears in the printed specification of the above numbered patent requiring correction and that the said Letters Patent should read as corrected below.

Column 3, line 71, and column 4, line 66, for "3-o-hydroxyphenyl", in each occurrence, read -- 3-p-hydroxyphenyl --.

Signed and sealed this 14th day of January 1958.

(SEAL)

Attest:

KARL H. AXLINE

Attesting Officer

ROBERT C. WATSON  
Commissioner of Patents